

July 8, 1958

L. A. OBERLY ET AL

2,842,473

PROCESS FOR COATING CLOTH

Filed June 15, 1955

2 Sheets-Sheet 1



Fig. 1



July 8, 1958

L. A. OBERLY ET AL

2,842,473

PROCESS FOR COATING CLOTH

Filed June 15, 1955

2 Sheets-Sheet 2



Fig. 4



Fig. 5

INVENTORS:  
LOUIS A. OBERLY  
CARL B. SALZINGER  
BY  
Thomas J. Mayner  
ATTORNEY

1

2,842,473

## PROCESS FOR COATING CLOTH

Louis A. Oberly, Chagrin Falls, and Carl B. Salzinger, Cleveland, Ohio, assignors to Industrial Rayon Corporation, Cleveland, Ohio, a corporation of Delaware

Application June 15, 1955, Serial No. 515,608

2 Claims. (Cl. 154—126)

This invention relates to a cloth coating process and has particular reference to a process for the coating of relatively open construction cloth materials employed as backing supports for subsequently applied film layers of a coating material.

Cloth or fabric, particularly of textile origin, is commonly utilized as a backing support for various coatings. Products suitable for clothing, Leatherette coverings, upholstery and decorating material and the like are advantageously manufactured from coated textile fabrics. Such products beneficially possess composite characteristics of the combined coating material and the backing cloth.

It has been found desirable to utilize resin-containing plastic materials as coatings for fabric. The coated fabric product may comprise a film layer of resin-containing plastic material, such as a vinyl polymer resin, applied over one surface of the backing cloth. Coated fabric products of this nature are characterized and known as supported films.

Suitable backing cloth for supported films may be a fabric of various construction. However, it is often advantageous to employ a knit cloth for such purposes. Knit cloth is generally more economical to construct than equivalent woven fabric. In addition, it has the advantage for many purposes of having substantially more uniform strength and extensibility in all directions.

Supported films are frequently utilized for applications where they are required to be sewn or stitched. For this purpose it is advantageous for the backing cloth to be only partially impregnated by the film layer of coating material which it supports. When the envelopment of the backing cloth by the film layer is not total or complete, the supported film is enabled to more distinctly retain certain of the desirable characteristics of a textile fabric, particularly with respect to tear resistance and the tear or sew line strength of the material in the vicinity of stitches. In addition, supported films have greater extensibility and resistance to permanent deformation upon elongation when the backing cloth is not completely enveloped.

When only one side of a cloth or fabric is being coated, it is sometimes difficult to control the extent of the penetration or impregnation of the coating material into the fabric to avoid excessive envelopment of the cloth backing by the supported film layer. This is more pronounced when a relatively open construction or mesh-like backing cloth, such as knit fabric, is employed. Control of penetration is difficult to maintain when relatively thin films, for example, those lighter than about 5 or 6 mils in thickness, are being applied. Such relatively thin coatings, particularly those having a thickness between about 0.5 and 3 mils, are often provided for coated cloth products which are intended to subsequently receive additional film layers of coating material.

When coating techniques are employed which utilize a casting belt of paper, metal or other relatively impervious material which is positioned under the backing cloth

2

as a support during the coating, there is a tendency for the coating material to penetrate or strike through the backing cloth. A greater degree of envelopment than is desirable may result. Should this occur, the supported film often displays poor resistance to tearing and an insufficient sew line strength for satisfactory application as a coated cloth product. In addition, its extensibility may be materially lessened.

It would be advantageous to manufacture supported films in a manner permitting close control of the degree of envelopment of the backing cloth by the film layer which it supports. It would also be advantageous to eliminate excessive penetration or strike-through of the coating material through the interstices of the backing cloth, especially when relatively thin film layers are being applied over open construction backing cloth. In this way, the production of supported film products having, among other desiderata, optimum tear resisting characteristics for purposes of stitching and sewing and an enhanced extensibility would be achieved.

It is among the objects of the present invention to provide a cloth coating process which permits close control of the envelopment of the backing cloth with the coating material and to also prevent undesirable strike-through of the coating material on the backing cloth. It is a further object of the present invention to provide a process wherein it is possible to simultaneously and economically produce both a supported and an embossed unsupported or sheet film product in the same operation.

These and other objectives and advantages are accomplished and realized in accordance with the present invention, by partially embedding and temporarily laminating the cloth to be coated with a sheet of a casting film; then applying a film layer of coating material over the unembedded or unlaminated side of the cloth; setting the supported film layer on the temporarily laminated cloth; and subsequently stripping the casting film from the uncoated side of the produced supported film.

Still further features and advantages of the present invention will be more apparent in the following description and the drawing, in which like reference numerals relate, insofar as possible, to like parts, wherein:

Figure 1 schematically portrays the coating process of the present invention;

Figure 2 schematically represents an embodiment of the process;

Figure 3 schematically illustrates a variation in the coating technique which may be employed in accordance with the present invention; and

Figures 4 and 5 schematically represent other embodiments of the process.

With reference to Figure 1, a backing cloth 10 is pressed into and partially embedded in a softened casting film 11 with which it is temporarily laminated while passing between a pair of pressure laminating rolls 12 and 14, rotated respectively in the direction of the arrows 13 and 15. The casting film 11 is a sheet or unsupported film which can be softened to permit the temporary lamination of the backing cloth. For example, solvents or plasticizers may be employed to condition the casting film to a suitable degree of softness. They may be present in the formed film or they may be purposely provided to accommodate the temporary lamination. Advantageously, however, the casting film 11 is a thermoplastic material, such as a vinyl polymer resin, which can be conditioned and softened by heat for the temporary lamination. In such cases it is advantageous for the pressure laminating rolls 12 and 14 to be heated to soften the thermoplastic casting film. While the casting film may be of any desired thickness, good results are obtainable with films having a thickness between about 18 and about 32 mils.

The backing cloth may be fabric of any material and construction. It may be a relatively open construction, mesh-like, scroopy or sleazy, material having substantially sized foramina or interstices. For example, loosely knit cloth of continuous filament viscose rayon yarn, having yields varying from about 10 to about 3 square yards per pound may advantageously be employed.

When thermoplastic casting film 11 is employed, the heated rolls 12 and 14 sufficiently soften it to permit the backing cloth 10 to be embedded in the casting film to a desired degree under the pressure of the rolls. If the casting film is a vinyl polymer resin, it is usually sufficient to heat it to a softening temperature of about 300° F. to 325° F. to partially embed and temporarily laminate the backing cloth. It is ordinarily advantages for the backing cloth to be embedded between about one-third to one-half of its thickness to effect the temporary lamination. The casting film is thus embossed with the structural pattern of the backing cloth. A temporarily laminated backing cloth 16 is formed as a first intermediate product in the process.

Roll pressures of about 100 to 1000 pounds and greater per square inch are usually sufficient for this purpose. The proper roll pressure in particular instances may depend on such various factors as the condition of softness of the casting film, the characteristics of the backing cloth, roll hardness and the speed of lamination. For example, good temporary lamination can be achieved within the mentioned pressure range at processing speeds of about 5 to 7½ yards per minute when using rubber cover rolls having a durometer reading of about 50.

Other suitable heating means (not shown) may also be employed to soften thermoplastic casting film for temporary lamination with the backing cloth. For example, before the cloth is pressed into the film between the rolls 12 and 14 or by other means, the film may be preliminarily brought to a softening temperature by being first passed over heated cans or rollers or over Calrod units. The preheating may also be accomplished through an oven or with infra-red radiation. In such cases the laminating rolls 12 and 14 may not require internal heating means for softening the casting film. They may then be merely employed as pressure rolls. However, when preheating is employed for softening the film, it may be advantageous to keep the pressure rolls warm to sufficiently maintain the softened condition of the film during the temporary lamination.

The unembedded side of the intermediate temporarily laminated backing cloth 16 is covered with a film layer of a desired coating material, such as a vinyl polymer resin. Any desired method of coating may be employed, including any of the various well-known techniques of spread or dispersion coating or coating by calendering techniques which are practiced in the art. In each instance the particular method utilized may vary with the specific coating materials being applied and the characteristics desired in the supported film product.

For purposes of convenient illustration, knife coating is depicted in Figure 1. The temporarily laminated backing cloth 16 is passed over a support roll 17, rotated in the direction of the arrow 18. A quantity of coating composition is supplied behind a knife or doctor blade 20 to maintain a pool 21 of the coating composition which is spread as a thin supported film layer 23 upon and over the upper unembedded surface of the backing cloth. A film of any desired thickness may be applied, depending upon the particular use anticipated for the coated cloth product. Strike through of the coating material is physically prevented by the casting film which is temporarily laminated to the backing cloth. The coating material is thus able to penetrate or impregnate the backing cloth only to a controlled depth equivalent to its unembedded portion in the casting film, regardless of the interstitial area of the cloth.

After application to the temporarily laminated backing

cloth 16, the film layer 23 of coating material is set or cured according to suitable conventional techniques for the particular coating material employed. This is accomplished in a curing, setting or drying zone 25 which is operated according to the requirements of the particular situation. For example, in order to cure or set many coating materials, heating or drying by means of heated air or other fluid, infra-red radiation or by other heat-exchanging contact or conducting means may be required. Most vinyl polymer resin compositions including emulsions, plastiols and organisols require sufficient heat to remove volatile constituents and to fuse or flux the resin to its finished form. If hot melt coating is being practiced, the curing or setting of the supported film layer may require that cooling means be employed.

The used casting film 10, having the pattern of the backing cloth embossed on its surface, is stripped from the uncoated side of the backing cloth 16 at a separation point 27. The supported film product 29, after being freed from the temporarily laminated casting film, is taken up for collection in any suitable fashion. For example, a wind up reel may be employed. The stripped casting film 11 may also be collected in any desired manner.

The process of this invention may be carried out with apparatus patterned after that schematically illustrated in Figure 2. A four-roll inverted L calender 30 may be employed to produce the casting film 11 for temporary lamination to the backing cloth 10. The calender 30 comprises a stack of rolls 32, 34, 37 and 40 revolving in close proximity to one another in the direction of the arrows 33, 35, 38 and 41 respectively. A suitable film forming material, advantageously a thermoplastic material such as a vinyl chloride resin composition, is supplied to the nip between the rolls 32, 34 to maintain a rolling bank 31 of resin therein. When thermoplastic materials are employed the rolls 32, 34, 37 and 40 in the calender stack are conveniently heated. The resin composition, according to conventional practice, is supplied from a mixer, such as a Banbury mixer or the like after being suitably compounded with plasticizers, fillers, stabilizers, etc. in blending apparatus. The film produced in the nip of the rolls 32, 34 follows around the roll 34 at 36 to the nip of the roll 37 with the roll 34. The film is reduced in the nip between rolls 34, 37 and follows around the roll 37 at 39 to the nip of the roll 37 with the roll 40. The film is further reduced in the nip between rolls 37, 40 and follows around the roll 40 at 42 from which the finished sheet of unsupported casting film 11 is delivered to the laminating rolls 12, 14.

As mentioned, the casting film may, if desired, be softened in any suitable manner prior to entering between the laminating rolls. Advantageously, a thermoplastic casting film is softened by preheating and the laminating rolls 12, 14 are heated. The backing cloth 10 is payed out from a supply reel 45 around a roll 46. It is pressed into the softened casting film under the pressure of the laminating rolls 12, 14.

The intermediate temporarily laminated backing cloth 16, comprised of the backing cloth 10 embedded in and temporarily laminated with the casting film 11, is passed from the laminating rolls 12, 14 around and under a roll 48, rotating in the direction of arrow 49, then around and over a roll 50, rotating in the direction of the arrow 51. The coating is applied to the temporarily laminated backing cloth 16 from the supply pool 21. It is spread over the open, unembedded surface of the backing cloth by the knife 20 on the upper side of roll 50. The supported film layer 23 of coating material on the temporarily laminated backing cloth 16 is passed over a consecutive pair of support rolls 52, rotating in the direction of the arrows 53, through a curing or drying zone 55. This sets the applied film layer on the supporting backing cloth.

When organisol or plastisol paste compositions of vinyl polymer resins are employed for coating, they may be dried and fused on the backing cloth with air at a temperature of between about 175° F. and 450° F., or by direct infra-red radiation from electrically heated elements at a source temperature of about 1000° F. to 2000° F.

The supported film, still temporarily laminated to the casting film, is passed around cooling rolls 58, rotating in the direction of the arrows 59. The embossed casting film is stripped from the supported film or coated cloth product 29 at the separation point 27 by the stripping rolls 61, 62 and 63. Ordinarily a pulling force of between about  $\frac{1}{4}$  pound and  $2\frac{1}{2}$  pounds per linear inch is sufficient to separate the casting film from the supported film product. The supported film 29 is passed around the rolls 65, 66 to be wound in a take-up reel 68. The stripped casting film is wound in a take-up reel 70.

In Figure 3 a reverse roll coater is employed to illustrate a calender coating or so-called "bank-skimming" technique to apply the supported film layer. The casting film 11, which for purposes of illustration is thermoplastic, may be conveniently supplied from a supply reel 42 of already formed unsupported film. It is temporarily laminated to the backing cloth 10 between the heated laminating rolls 12, 14. The casting film may be formed in any desired manner including calendering or extrusion. Also, as illustrated, it may be produced in advance of requirements for its temporary lamination with the backing cloth. The temporarily laminated backing cloth 16 is passed under and around the roll 48, rotating in the direction of the arrow 49, then over the roll 50, rotating in the direction of the arrow 51. Coating material is applied from the roll 76 after being formed as a film between the rolls 74, 76. A rolling bank 72 of the coating material is maintained in the nip of the rolls 74, 76, rotated respectively in the directions of the arrows 75, 77. The film to be applied follows around the roll 77 at 78. It is literally wiped onto the unembedded surfaces of the temporarily laminated backing cloth 16, moving in a direction opposite to the roll 76. The film layer 23 is then set as a supported film product on the backing cloth. The embossed casting film 11 is subsequently stripped away and separated from the supported film product.

Embossed casting film may, if desired, be reclaimed for re-use in the production of fresh casting film. This may be accomplished by remelting or recompounding the used casting film for formation of fresh film through calendering or other film forming techniques. In addition, it is possible to smooth the embossed surface of used casting film by means of heated pressure resurfacing rolls in order to make it more suitable for additional temporary lamination whenever an absolutely smooth surfaced casting film is necessary or desirable. In this way, greater service may be obtained from a given quantity of casting film before reclamation or other disposal is necessary.

Advantageously, however, the used casting film may be employed as an embossed unsupported film product having the structural pattern or design of the impressed backing cloth on its surface. An economic benefit may thus be realized in the process since both a coated cloth or supported film product and an embossed sheet or unsupported film product are simultaneously manufactured. If desired, the embossed, unsupported film product may be pressed onto a backing cloth to form an embossed, supported film. Or both surfaces of the casting film may be employed for the temporary lamination to the backing cloth before it is either reclaimed or disposed of as an embossed film.

The casting film, especially if it is of a thermoplastic nature, may also be employed as a continuous belt. This eliminates the necessity to take up used casting film after it is separated from the supported film. As shown in Figure 4, the casting film 11 is passed as a continuous belt

around the plurality of rollers 70, rotating in the direction of the arrows 71. The backing cloth 10 from the supply reel 45 is embedded in the belt of casting film between the heated laminating rolls 12, 14. The unembedded side of the temporarily laminated backing cloth 16 is coated with material from the supply pool 21 spread by the knife 20 on the upper side of roll 50, rotating in the direction of the arrow 51. The supported film layer 23 on the temporarily laminated backing cloth 16 is passed under a drier 55 to set the applied film on the cloth. The intermediate temporarily laminated supported film product is then cooled between the cooling rolls 59, rotating in the direction of the arrows 58, or by other suitable cooling means. The supported film product 29 is separated from the continuous belt casting film 11 with the separating roll 62. It is collected on the take-up reel 68.

When utilizing casting film as a continuous belt, it may be advantageous to employ belt tensioning means to counteract any slack that may develop. Additional heated pressure rolls may also be advantageously employed to smooth the embossed surface of the casting film after its temporary lamination. In addition, supplemental coating means may also be employed to maintain a predetermined casting belt thickness in order to overcome any attenuation that may develop as a result of belt passage around and between the various rollers.

As is illustrated in Figure 5, these features, when desired, may be added to the basic continuous belt arrangement of Figure 4. The continuous belt of casting film 11, after being stripped from the supported film product 29, is passed around a "floating roll" belt tensioning means 36 positioned between the rolls 35, 37. The tensioning means 36, as shown, consists of a counterweighted vertically movable roll around which the belt passes. Of course, other suitable belt tensioning means may also be employed. If attenuation and belt elongation becomes greater than can be compensated for by a belt tension device, it may become necessary on occasion to cut and splice the casting film belt.

A pair of heated pressure rolls 80 and 82, rotating in the direction of the arrows 81, 83, may be utilized to smooth the surface of the thermoplastic casting belt from impressions of the backing cloth which are embedded therein during the temporary lamination. The supplemental coating means for the belt of casting film may be a reverse roll coater, as depicted, comprising the rolls 92, 94 rotating in the direction of the arrows 93, 95. A desired additional thickness of coating material is applied from the rolling bank 96 of film forming material in the nip of the rolls 92, 94 to the surface of the casting film 11 while it is passing over the roll 90, rotating in the direction of the arrow 91. Other supplemental coating means may also be employed for maintaining the thickness of the casting belt.

The surface of the casting film may, if desired, be treated or prepared with various agents to facilitate stripping and separation from the supported film product. Treatment with such agents may, as desired, be effected before or after the casting film is conditioned or softened for temporary lamination with the cloth, although it is frequently more convenient to do so before softening the film. Finishes which contain commonly known partitioning agents may advantageously be applied for this purpose before the casting film is temporarily laminated with the backing cloth. For example, certain hydrophobic and hydrophilic colloids including those selected from the group consisting of silicones, stearates and some of the alkali metal salts of higher melting point fatty acids may be so employed. Also where the required time and temperature conditions for curing the applied finish would not be deleterious to the casting film, certain urea formaldehyde, phenol formaldehyde and like compounds and derivatives may be employed.

The casting film may be of any film forming material, preferably thermoplastic, capable of being formed or

worked into unsupported sheets and conditioned for temporary lamination to the backing cloth. Advantageously, as mentioned, the casting film comprises a composition which essentially contains a vinyl polymer resin, such as a vinyl chloride resin or copolymers of vinyl chloride and other ethylenically unsaturated compounds, well-known to the art.

Likewise, the coating may be of any suitable material. While vinyl polymer resins are most advantageously employed, the coating material may also comprise polymeric substances of a varying nature including polyamide and polyester type materials well-known in the art. Suitable coating materials of any origin, capable of being spread or calendered over backing cloth and formed into a supported film product, may be employed in the process of the present invention.

The coated cloth or supported film product may receive subsequent coatings, if desired. Supported films of any desired thickness may be produced in accordance with the present invention.

The applied coating may also serve as an adhesive layer or "anchor" coating for subsequent application through calendering or lamination of an additional, already-formed sheet or unsupported film of desired material, such as an unsupported sheet of a vinyl polymer resin. In such cases, as mentioned, it is advantageous for the coated cloth product to have a film thickness between about 0.5 and 3 mils.

The invention may be better understood by reference to the following examples and description in which all parts, unless otherwise indicated, are by weight.

#### Example I

A casting film composition was compounded containing about 100 parts of a substantially pure polyvinyl chloride resin; about 20 parts of dioctyl phthalate as a primary plasticizer for the film; about 12 parts of dioctyl sebacate as a low temperature plasticizer; about 10 parts of tricresyl phosphate as a flame proofing plasticizer; about 4.5 parts of a stabilizer comprising a mixture of a barium cadmium soap, an epoxy compound and a chelating (sequestering) agent; about 15 parts of calcium carbonate filler; and about 0.25 part of triple pressed stearic acid as a lubricant. The ingredients, after being blended, were mixed in a Banbury mixer and dumped at a temperature of about 310° F. Casting film having a thickness of about 20 mils was produced on a four-roll inverted L calender operated at a temperature of about 320° F.

A backing cloth of about 3 ounces per square yard circular knit viscose rayon cloth was pressed into the casting film at a rate of about five yards per minute between a pair of heated laminating rolls. The film was warmed to a softening temperature of about 320° F. which facilitated partially embedding the cloth to about half its depth in the film under the pressure of the rolls. The effective roll pressure for the temporary lamination of the backing cloth with the casting film was about 250 pounds per square inch.

A plastisol coating composition was spread coated with a doctor knife on the unembedded side of the temporarily laminated backing cloth. The plastisol was formulated with about 100 parts of a copolymer dispersion resin containing about 95% by weight of vinyl chloride copolymerized with vinyl acetate; about 75 parts of dicapryl phthalate as a primary plasticizer; about 3 parts of a heat and light stabilizer containing a suitable metallic soap, an epoxy compound and a chelating agent; about 4 parts of a suitable viscosity depressant; and about 20 parts of a calcium carbonate filler. The applied coating composition forming the supported film layer had an average approximate thickness of about 7 mils. The plastisol was set in a drying oven at a temperature of about 300° F. which fused the film on the backing cloth.

After the cured supported film coating was cooled, the temporarily laminated backing film was stripped from

the coated cloth product. The surface of the used casting film was embossed with the design of the knit backing cloth. It made a suitable embossed unsupported vinyl film product which could be further pressed to backing cloth to produce an embossed supported film.

The adhesion strength of the supported film on the backing cloth was at least about four pounds per inch wide strip. The coated cloth product had a desirable minimum tear strength of about five pounds. Its stitch tear strength (as measured by the pulling force required to separate two pieces sewn together with about 12 stitches per inch) was about eighty pounds in the lengthwise direction and about fifty pounds in the cross direction. It had good extensibility, retaining not more than about 1½% permanent stretch in any direction after being pulled with about a ten pound force for about ten minutes.

#### Example II

A casting film was compounded and formed as described in Example I excepting that octyl decyl phthalate was employed as the primary plasticizer and the film was calendered to a thickness of about 30 mils. A backing cloth of about 5.3 ounces per square yard circular knit viscose rayon cloth was temporarily laminated with the casting film according to the procedure set forth in Example I. The temporarily laminated backing cloth was reverse roll coated with the plastisol composition as described in Example I with the exception that about 20 parts of a color pigment was incorporated in the plastisol formulation. The applied coating had a thickness of about 15 mils. The coated cloth product, after being stripped from the casting film, displayed excellent properties. The adhesion strength between the supported film and the backing cloth was about four and one-half pounds. Its tear strength was at least about five pounds. Its stitch tear strength was about ninety pounds longitudinally and about sixty pounds crossways.

The extensibility of the coated cloth was equivalent to that described in Example I.

The used casting film was reclaimed by being remelted, mixed in a Banbury and then recalendered into fresh film. Coated cloth produced on reclaimed casting film had characteristics and properties equivalent with that described above.

#### Example III

The coating procedure of Example I is followed excepting that the backing cloth employed for supporting the coating is a 3 ounce per square yard woven 64 x 54 thread count viscose rayon fabric. The properties of the coated cloth product are about equivalent to those described in Example I excepting that the extensibility of the material, due to the nature of the backing cloth, is not uniformly as good in all directions.

#### Example IV

The coating procedure of Example I is repeated on a 2 ounce circular knit viscose rayon cloth excepting that the applied supported film layer has a thickness of only about 2 mils. After the supported film product is separated from the casting film, it is pressed to an unsupported vinyl film which is laminated to the plastisol coating on the backing cloth. The final supported film product weighs about 24 ounces per square yard. The adhesion strength of the film layer to the backing cloth is about four and one-quarter pounds. Its strip tear strength is at least about five pounds and its stitch tear strength about eighty pounds lengthwise and about fifty pounds across. The extensibility of the supported film product is good. The material does not retain more than about 1½% permanent stretch in any direction after it is pulled with about a ten pound force for about ten minutes.

#### Example V

The coating procedures of Examples I, II and III are repeated using the unembossed side of a previously used casting film for temporary lamination with the backing

cloth. The coated products obtained have properties which are commensurate with those described in the first three examples.

*Example VI*

The coating procedures of Examples I, II and III are repeated excepting that the casting film is formed and employed for substantial periods as a continuous belt. The backing film is temporarily laminated with the moving continuous belt on which its unembedded side is coated. After the supported film product is stripped from the belt, the embossed surface produced from the temporary lamination of the backing cloth is smoothed between heated pressure rollers before the film is returned to be further temporarily laminated with uncoated backing cloth. The coated products obtained have properties corresponding to those described in the first three examples.

Since certain changes and modifications may readily be entered into in the practice of the present invention without substantially departing from its intended spirit or scope, it is to be understood that all of the foregoing be interpreted and construed as being merely illustrative and in no sense or manner limiting of the invention, as particularly pointed out and defined in the appended claims.

What is claimed is:

1. Process for coating cloth on a moving belt of thermoplastic casting film which comprises passing said belt of casting film through heat softening means; partially embedding cloth under pressure in the softened portion of said moving belt of casting film to temporarily laminate said cloth with said belt; applying a film layer of coating material over the unembedded side of the cloth while it is temporarily laminated with said moving belt of casting film; curing the applied film layer of coating material on the cloth while it is temporarily laminated with said moving belt of casting film; separating the coated cloth from the moving belt of casting film; maintaining

said moving belt of casting film under a substantially constant tension; and smoothing the surface of said moving belt of casting film to remove cloth impressions after the belt is separated from said coated cloth before returning through the said heat softening means.

2. Process for coating cloth on moving belt of thermoplastic casting film which comprises passing said belt of casting film through heat softening means; partially embedding cloth under pressure in the softened portion of said moving belt of casting film to temporarily laminate said cloth with said belt; applying a film layer of coating material over the unembedded side of the cloth while it is temporarily laminated with said moving belt of casting film; curing the applied film layer of coating material on the cloth while it is temporarily laminated with said moving belt of casting film; separating the coated cloth from the moving belt of casting film; maintaining said moving belt of casting film under a substantially constant tension; smoothing the surface of said moving belt of casting film to remove cloth impressions after the belt is separated from said coated cloth and before returning through said heat softening means; and applying additional quantities of casting film forming material directly on said belt to maintain it at a predetermined thickness.

25

References Cited in the file of this patent

UNITED STATES PATENTS

|           |                 |               |
|-----------|-----------------|---------------|
| 1,634,710 | Crowell         | July 5, 1927  |
| 2,193,496 | Schwartz et al  | Mar. 12, 1940 |
| 2,442,443 | Swallow         | June 1, 1948  |
| 2,444,094 | Duggan          | June 29, 1948 |
| 2,595,127 | Coffey          | Apr. 29, 1952 |
| 2,618,580 | Lancaster       | Nov. 18, 1952 |
| 2,700,630 | Bukey et al     | Jan. 25, 1955 |
| 2,706,699 | Plansoen et al. | Apr. 19, 1955 |
| 2,723,962 | Hedges et al.   | Nov. 15, 1955 |